

P. GERMAIN.

PROCESS OF SEPARATING METALS FROM ORES.

APPLICATION FILED AUG. 3, 1908.

921,227.

Patented May 11, 1909.



Inventor

Pierre Germain

G. Gittman.

Witnesses

J. P. Britt  
Hugo Glare

By

Attorney

# UNITED STATES PATENT OFFICE.

PIERRE GERMAIN, OF PARIS, FRANCE.

## PROCESS OF SEPARATING METALS FROM ORES.

No. 921,227.

Specification of Letters Patent.

Patented May 11, 1909.

Application filed August 3, 1908. Serial No. 446,801.

*To all whom it may concern:*

Be it known that I, PIERRE GERMAIN, a citizen of the Republic of France, residing in Paris, in the Republic of France, have invented certain new and useful Improvements in Processes of Separating Metals from Ores, for which application has been made in France, August 14, 1907, Germany, November 18, 1907.

10 This invention has for its object a process for separating precious and other metals, which are combined with their gangue or inclosed therein, from their ores.

An apparatus is shown diagrammatically 15 in section in the accompanying drawings as an example of construction, which apparatus may be employed for carrying out the process.

This apparatus consists of a boiler (autoclave) 1, which may be made of enameled 20 cast iron or steel and which can be exposed to an internal pressure of approximately 100 atmospheres with sufficient safety of working. In the direction of the central axis of this pressure boiler there is a steel tube 2,

25 through which steam is admitted from an inlet pipe 15 at a pressure of about 20 atmospheres. The steam admitted through this tube transmits its heat to the ore to be treated and also to the reagents which are thoroughly mixed with the ore, and thus are in contact with it on all sides. A stirring mechanism, formed of a hollow shaft 3 which is provided with a large number of apertures 3' in order to admit the ores and the reagents 30 in contact with them, which flow around the pipe 2, and which has also arms or blades 4 which have the form of a spiral segment or any other form, serves for thoroughly mixing the mass to be treated. The upper and lower

40 ends of the shaft 3 of the stirring mechanism run in annular bearings 5. The stirring mechanism receives its motion, for instance from a belt pulley 6 which is keyed on the end of a shaft 7 which is passed through the

45 lower part of the pressure boiler and is formed in one piece with the hollow shaft 3. A suitable stuffing box is preferably employed for obtaining the necessary tight joint. The pressure boiler 1 is also provided 50 with a feed aperture and a suitable pipe 8 for introducing the fluid, also with a manometer 9, one or more thermometers 10, a drawing off and decanting side tap 11 and a pipe 12 which serves for conveying the gases into two

absorption vessels arranged beneath the apparatus.

In addition to the hereinbefore mentioned apparatus, other independent organs and apparatus are used during the treatment of the ores, which apparatus serve for filtering the 60 solutions obtained when drawn off and also for washing and separating the ores from their solutions. All these arrangements and parts and also the pressure boiler are enameled internally, in order that they may remain protected against the decomposing and 65 corroding action of the acids.

In order to allow the pressure boiler to be conveniently fed and discharged, it is preferably arranged so as to tilt and rock after 70 the manner of the Bessemer converter. For this purpose the pressure boiler holder is provided in its central part with two pins 13 lying opposite one another, which are carried by two suitable bearing frames or brackets 75 14. A suitable device is also provided for fixing the pressure boiler in a suitable position.

The pins 13 are made hollow, in order to allow of the passage of two pipes 15 and 16, 80 one of which 15 serves for introducing high pressure steam to the vertical internal pipe 2, while the other 16 is intended for admitting the active solutions and re-agents under pressure into the pressure boiler. The 85 means for tightly packing or fitting the pipes 15 and 16 relative to the hollow pins 13 may be any suitable ones. A fundamental condition is however that it must remain possible to tilt on its axis and even to completely 90 reverse the pressure boiler.

The feed and introduction of the ore to be treated into the pressure boiler, and also the discharge of the residues takes place through a man-hole 17, which is closed by a suitable 95 man-hole cover 18.

The pressure in the interior of the pressure boiler is obtained in any suitable way. This is, however, preferably produced by means of a suction and pressure pump, which is 100 enameled internally and also serves for conveying, through the steam pipe 16, a concentrated solution of sodium hypochlorite into the pressure pump.

In order to treat the ore I proceed in the 105 following way:—The ore is first thoroughly cleaned by removing the worthless constituents, such for instance as silica, carbonate of

lime and magnesium, iron oxids etc. The hard silica and the quartz are removed by disintegration by means of resilient and yielding grindstones and also by sifting. 5 The calcium and magnesium carbonates, and also the alumina, are removed by cold washing by means of dilute hydrochloric acid. Finally the iron oxids are also removed (cold) by means of dilute sulfuric acid. 10 The precious metals are not affected by any of these washing processes. The ore treated in this way is also freed from the extracting and washing residues and also from the moisture contained therein. The 15 weight of the ore is now reduced 9/10 that is to say there remains only 1/10 available. This remaining ore is now treated with very finely subdivided iron so-called chemically pure iron, which is obtained as is well known 20 by calcining and roasting iron oxid in the presence of very finely sub-divided charcoal in a closed vessel. The ore mixed in this manner with the re-agent is now introduced into the pressure boiler, which at this moment 25 is in a horizontal position, and directly afterward hydrochloric acid is introduced through the pipe 8. The stirring mechanism 3, 4, is now set going and the ore is subjected to the action of heat, steam being admitted 30 through the center pipe 2. After a little time a concentrated solution of sodium hypochlorite is introduced under pressure by means of the pump, through the pipe 16. Under the action of the pressure existing in 35 the interior of the pressure boiler and the heat, hydrogen is generated therein, which at the considerable pressure and the high temperature reduces the sulfids, arsenids, tellurids, selenids. At this moment nitric acid 40 is introduced under pressure in a quantity which is so calculated as to form with the excess of hydrochloric acid aqua regia. The reduced metals in *statu nascendi* are now dissolved by the aqua regia contained 45 in the pressure boiler, which is also exposed to the action of heat and pressure. There then escapes sulfureted-arseniureted, tellureted and so-forth, -hydrogen, also chlorin in a nascent condition at a considerable 50 pressure and high temperature. There is also formed nitrates of copper, tin, bismuth, cobalt according to the kind of ore treated, and also simple or alkaline chlorids of gold, platinum, silver, uranium, sodium and the like. 55 The sodium-containing residue, which is derived from the combination of the excess sodium hypochlorite with the nitric acid which is also in excess, consists of chlorid of sodium or common salt, which combines with the metallic chlorids and renders them 60 soluble under heat. Without this reaction, which induces the formation of a soluble double chlorid, the chlorid of silver would be lost by reason of its insolubility. 65 After the three-fold action of the high pres-

sure (50-60 atmospheres), the high temperature (250-300° C.), and the hydrogen in a nascent condition (*status nascendi*), which is produced by the action of the finely sub-divided iron on the free acid, has been continued for a sufficient time, the pressure boiler is again brought into its vertical position and the solutions are then drawn off and decanted, the tap 12 is then opened which leads to the small containers which are intended for the absorption and reception of the free gases contained in the pressure boiler 70 1. The first of these vessels which is not shown in the drawings, contains a hydrocarbon, for instance, turpentine oil or the like, for the purpose of absorbing the chlorin; further in the second vessel ammonia solution is contained, to dissolve the nitrogen derivatives. The sulfureted, arseniureted, tellureted and so forth hydrogen, is then 75 passed in succession through the two vessels and is consumed by means of a separate burner arranged for this object.

The decanted and drawn off solutions are run off through suitably arranged taps, these 90 taps being situated somewhat beneath the level or the surface of the ore treated. Further the liquid is filtered through a filter press arranged outside the pressure boiler. Steps are also taken for a thorough washing 95 of the residual ores and the water resulting from the washing and extraction is treated like the filtered solutions.

According to the chemical constitution of the ore treated, the presence of copper-, tin-, 100 cobalt-, bismuth-, etc., nitrate, or a silver- and sodium- double chlorid or gold-, platinum-, iridium-, uranium-, radium-, chlorid or the like, may be ascertained.

The solutions removed from the pressure 105 boiler are concentrated in any suitable way and exposed to the action of electric currents of suitable potential for the purpose of electrolysis by the usual methods.

Of course the above process may not only 110 be employed for ore residues, but also for all ores of similar constitution or analogous formation.

I declare that what I claim is:

1. A process for treating metallic ores, 115 consisting in mixing the ore with disintegrated iron, introducing the mixture into a pressure boiler, treating the mixture in said boiler with hydrogen and chlorin in a nascent condition, which gases reduce the metallic 120 compounds, and adding nitric acid to the mass so that all resultant metals are attacked in order to yield soluble double nitrates or chlorids.

2. A process for treating metallic ores, 125 consisting in mixing the ore with disintegrated iron, introducing the mixture into a pressure boiler, treating the mixture in said boiler under the action of heat and pressure with hydrochloric acid and then with sodium 130

hypochlorite, which cause the generation of hydrogen and chlorin in a nascent condition, which gases reduce the metallic compounds, and adding nitric acid to the mass so that all 5 resultant metals are attacked in order to yield soluble double nitrates or chlorids.

In witness whereof, I have hereunto signed

my name this 21st day of July 1908, in the presence of two subscribing witnesses.

PIERRE GERMAIN.

Witnesses:

ANTONIN MONTEILBET,  
H. C. COXE.